

## UNITED STATES PATENT OFFICE

ALBERT L. CLAPP, OF DANVERS, MASSACHUSETTS

## LINER BOARD OR PAPER

No Drawing.

Application filed December 22, 1922. Serial No. 608,579.

In the manufacture of paper or card-board of the kind known commercially as "patent coated," such as used in the manufacture of cartons, boxes, containers and for other uses, it is customary by a suitable coating machine to apply to a sheet of formed and dried paper or board, a surface coating of china clay, blanc fixe or other surfacing material, and casein or other like adhesive.

10 The object of the invention is to provide a liner paper or board having a surface coating of china clay, blanc fixe or other equivalent material to impart a smooth or satiny finish, and to produce the same at one operation in 15 a paper machine.

I have made the discovery that kieselguhr or "cellite," and wood flour, either separately or in combination, have the property or capacity, when suspended in water, of being 20 "formed" on the cylinder mold of a paper machine and of being transferred to a make-up roll or blanket thereof, although the layer or layers thus placed or built up on the make-up roll or blanket cannot be removed as a 25 web or sheet as they have no tensile strength. I have also discovered that these two substances also have the property of carrying with them a large or dominant quantity of 30 china clay, blanc fixe or other pulverulent coating materials. As a result of these two discoveries, I have found from prolonged experimentation that it is possible to apply to a layer of paper or board, while it is being 35 formed and is still in a wet state, a layer of cellite or wood flour or both, and the previously-mentioned coating materials, so that, when the composite sheet is dried, it possesses the desirable characteristics of the "patent coated" paper or board.

40 In carrying out my invention, I use a multiple-cylinder paper machine having the proper vats associated with the several cylinders and transfer rolls. In one of the vats I place any suitable paper stock such as may 45 be required for producing the desired paper

or board, and in another vat I place an aqueous suspension of cellite and/or wood flour and a dominant proportion of the desired filler or coating substance. Then to the wet web of the paper stock, transferred to the 50 blanket or belt of the machine, I apply a layer of the stock in the second vat, or vice versa, so that a composite web or sheet is formed which is dried in the usual manner, with the 55 result that the finished product has an adherent top surface or layer of the coating substance.

In carrying out my invention, one may proceed as follows: In a beating engine, I prepare a suitable pulp by vigorously beating together 50 parts, by weight, of mixed waste paper and an equal amount of bleached sulphite pulp. When this has been accomplished, I add 5 parts of rosin size, and, when this has been thoroughly "brushed" 60 into the pulp, I add 5 parts of alum and continue the beating until reaction has been accomplished. In another beating engine I place 10 parts, by weight, of cellite or kieselguhr, 20 parts of wood flour, and 70 parts of 65 china clay, together with water to form a suspension. These are beaten or agitated until a suspension is produced which will "form" 70 on the cylinder mold of a paper machine. Then into two separate vats of a multiple-cylinder paper machine are placed the stocks produced as hereinbefore provided, and a composite web is formed consisting of a layer or web of fiber and a facially contiguous adherent layer of kieselguhr-wood flour-clay 75 mixture. The wet web or sheet is now treated in the usual manner followed in the manufacture of paper, being dried, calendered and wound into rolls. On being dried and calendered, the sheet has a surface layer comprising about 70% of china clay and 30% of the carrier.

Obviously it is unnecessary that the fibrous lamination or bottom layer of the fibrous sheet should be sized, and consequently, in

the formation of the pulp, the size may be omitted. Again, I should not regard it as a departure from the invention if the top layer should contain some fibers and/or a size. 5 Thus, in the formation of the stock for the top layer, I may use:

- 5 to 20 parts bleached sulphite pulp,
- 10 to 20 parts wood flour,
- 10 to 20 parts cellite,
- 10 50 to 70 parts china clay,
- 10 parts silicate of soda (or rosin size),
- 5 parts alum.

In such case, one may vigorously beat together in a beating engine the sulphite pulp 15 and the wood flour with water for about an hour, after which the cellite and the china clay are added and the stock beaten for a further period of about 30 minutes. Then the silicate of soda is thoroughly incorporated 20 in the stock, and finally the alum is added, after which the stock is "brushed out" for about an hour. The sodium silicate or sodium resinate is precipitated as aluminum silicate or aluminum resinate by the 25 alum, and constitutes a gelatinous size which coagulates and assists in retaining the china clay.

Of course I do not limit myself to the use 30 of china clay in the formation of the top layer, as any equivalent pulverulent material may be used, such, for example, as blanc fixe, pulverized rosin or carbon black, or other finely powdered pigments.

A composite sheet as herein described 35 "forms" perfectly and the laminations or layers adhere or interlock most satisfactorily.

I am not familiar with any generic name, other than the term "carrier" or words of similar import, which can be applied to wood 40 flour and kieselguhr or cellite. Either of these materials or both in combination have the properties hereinbefore described of "forming" on the cylinder mold and of being transferred as a continuous layer to the 45 blanket or felt of a paper machine and act as carriers in carrying or absorbing many times their weight of pulverulent material in their "formation." Due to the lack of a better term, I desire to have it understood that in 50 the claims, whenever I refer to "carrier" I mean either kieselguhr or wood flour alone or in admixture.

I also desire to be understood that the bottom fibrous layer of the composite web or 55 sheet may be made of any approved fibrous or cellulosic materials (sized or unsized as occasion demands) which it may be desired to use in the formation of any predetermined form of board or paper, the examples which 60 I have herein given being illustrative of composite webs embodying the invention and of the new or improved process which may be practiced in their production.

While I have herein referred to the use of 65 wood flour, which is a finely-disintegrated

product produced by grinding wood to a degree of fineness approximating wheat flour, nevertheless I would not consider it a departure from the spirit and scope of the invention if one were to use wood less finely ground. Thus, for example, I may substitute for wood flour finely-divided sawdust capable of passing through a 40 to an 80 mesh sieve, for I find that a product of this character has the property of "forming" on a cylinder mold, although in my opinion the results are not quite as satisfactory when finely-divided sawdust is used as when wood flour is used. 70

It is further obvious that, while I have referred to an exterior layer of china clay or blanc fixe, carbon black, or finely-divided pigments, the process as herein described includes the use of any finely-divided or pulverized material of the character of resins, pigments, gums or the like; so that, in referring to a "pulverulent material such as china clay or the like," I mean to include pulverulent substances of the character of all of those herein referred to which it may be desired to employ in the formation of the top layer of the sheet. 80

What I claim is:—

1. A composite sheet comprising a bottom layer of cellulosic material, and a top layer 95 comprising a mixture of pulverulent coating material, and kieselguhr.

2. A composite sheet comprising a bottom layer of cellulosic material, and a top layer comprising a mixture of a small proportion 100 of kieselguhr and a dominant proportion of pulverulent coating material.

3. A composite sheet comprising a bottom layer of cellulosic material, and a top layer comprising a mixture of a small proportion 105 of kieselguhr, a precipitate, and a dominant proportion of pulverulent coating material.

4. A process of producing a sheet having a surface layer of a pulverulent material, which comprises forming a web of pulp, independently forming a substantially non-fibrous web from an aqueous suspension of the pulverulent material carried by a finely divided carrier, and applying it as a contiguous adhering layer to said web of pulp, 110 and then simultaneously removing the water 115 from both webs.

5. A process of producing a sheet having a surface layer of a pulverulent material, which comprises forming on independent 120 cylinder molds and uniting a web of cellulose pulp and a substantially non-fibrous web of pulverulent material carried by a finely divided carrier capable by itself of forming on the cylinder mold, and drying the sheet. 125

6. A process which comprises forming into contiguous, adherent webs on a multiple cylinder machine, a web of cellulose pulp and a substantially non-fibrous web of a fine- 130 divided material carrying a preponderant

proportion of pulverulent material, and drying the sheet thus produced.

7. A process which comprises forming into contiguous, adherent webs on a multiple cylinder machine, a web of cellulose pulp and a substantially non-fibrous web of a finely divided material carrying a size and a preponderant proportion of pulverulent material, and drying the sheet thus produced.
- 10 8. A process which comprises forming into contiguous, adherent webs on a cylinder machine, a web of cellulose pulp and a web comprising only a small portion of fibrous material, size, and a finely divided material, carrying a preponderant proportion of a pulverulent material; and drying the sheet thus produced.

9. A process of producing a paper having a surface layer of pulverulent coating material, which comprises forming a web of pulp, independently forming a substantially non-fibrous web of kieselguhr carrying a preponderant proportion of the coating material, applying said second-mentioned web 25 as a continuous adherent layer to the web of pulp, and drying the web.

10. A composite sheet comprising a bottom layer of cellulose fiber, and a top layer comprising a mixture of china clay and 30 kieselguhr.

In testimony whereof I have affixed my signature.

ALBERT L. CLAPP.

35

40

45

50

55

60

65